

## UNITED STATES PATENT OFFICE

2,643,770

## FLOTATION OF MICA WITH SULFONATES

Elmer William Gieseke, Fountain City, Tenn., assignor to American Cyanamid Company, New York, N. Y., a corporation of Maine

No Drawing. Application November 26, 1949,  
Serial No. 129,704

5. Claims. (Cl. 209—166)

1

The present invention relates to the concentration of mica by froth flotation. More particularly, it concerns an improved anionic reagent combination for the froth flotation of mica. The invention contemplates both the reagent combination and the improved process of flotation using the combination.

There exists a marked commercial demand for micas for various purposes. While mica is one of the most common mineral types in the earth's surface, deposits sufficiently free from quartz, for various commercial purposes, are not readily found. Accordingly, various attempts have been, and are being, made to beneficiate mica by froth flotation to obtain mica concentrate of saleable grade.

In this connection, the use of the terms "mica" or "micas" is intended generally to cover various minerals, particularly muscovite, lepidolite, biotite, and vermiculite. As used in the present specification and claims, these terms are so intended.

Mica, being acidic, is conventionally beneficiated by the use of cationic-type flotation agents. Generally, these comprise mixtures of long-chain fatty acid amines, averaging about 12-20 carbon atoms in the aliphatic portion of the fatty acid residue. These must be supplemented ordinarily by use in conjunction with sulfuric acid and an aluminum salt such as alum or aluminum chloride.

Although in many cases acceptable concentrates can be obtained, the practice is not wholly satisfactory for a number of reasons. In many cases, the ratio of concentration is not sufficiently high. In many cases, due to the expensive reagent used, control must be maintained with excessive care. Further, because of the sensitivity of the cationic agents to slimes, ore pulp must be carefully deslimed. Still further, the choice of the amount of selected reagent to be used must be carefully made and maintained because of the ability of the amine to float quartz, as well as the silicates. Supplemental agents, usually aluminum salts, were required for this purpose. Last, but not least, the overall operation was more expensive than was generally considered desirable.

It is, therefore, the principal object of the present invention to provide a froth flotation process, which is not subject to these limitations. The reagents used should not be particularly expensive. Supplemental aluminum salts should not be essential. The degree of care required in their use should not be excessive. The process should not be unduly sensitive to the presence of slimes in the ore slurry being treated.

5

Surprisingly, in view of the nature of the mineral being concentrated, these objects have been accomplished by a flotation using an anionic reagent in an acid circuit. In addition to the acidic material, the reagents used comprise sulfonated petroleum hydrocarbons, preferably supplemented by a commercial diaryl dithiophosphate. The successful accomplishment of the desired objects in an anionic circuit, with these reagents, is particularly surprising, in view of the past use, considered necessary in the art, of commercial cationic-type reagents in cationic flotation.

10

So far as conditions of acidity are concerned, the requirements are not too restrictive. It has been found that successful results can be produced under conditions at which the pH value is about 6.0 or less. There is no particular advantage in going below a pH of about 2.5, although there is no particular harm in so doing. Substantially any acid-forming substance, capable of producing the desired pH conditions, may be used. Commercially, however, this is substantially limited to the use of inorganic mineral acids, particularly sulfuric acid. The latter, because of its general availability, is to be preferred. Hydrofluoric acid, on the other hand, should be avoided since this acid exerts a depressing effect on mica when using the promoters of the present invention.

20

Sulfonated petroleum hydrocarbons, such as those which constitute the principal reagent in carrying out the novel process of the present invention, are commercially available in a number of different forms. However, as shown, for example, in U. S. Patent 2,331,049, their principal source is as by-products from the refining of petroleum lubricating oil fractions in the course of treatment with fuming sulfuric acids or sulfuric acids. When so produced, these by-products are generally found to be salts of the sulfonated hydrocarbons. Most commonly, the metallic radical of the salt is sodium. However, salts of other metals, such as the alkaline earth metals, aluminum, and the like, are encountered. In some cases, no attempt has been made to neutralize the acid product. Even after neutralization, free sulfonates and/or sulfates are often found.

25

So far as the present invention is concerned, it makes little difference whether the sulfonated petroleum hydrocarbon is used per se or as a salt; whether or not the sulfur is present in a sulfate or a sulfonic group, there usually being some of both present; or whether the compounds are used as salts of sodium, potassium, calcium, barium, aluminum, and the like. Nor need the materials

be purified, since mixtures of compounds produce wholly satisfactory results. As used in the present case, the term "sulfonated petroleum hydrocarbons" is, therefore, intended to include such mixtures as are found in the commercial products.

Petroleum sulfonates, or derivatives thereof, which are suitable for use according to the process of the present invention are commercially available under a variety of designations. Among these found to be useful are "Petronate" and "O-Emulsifier," obtainable from L. Sonneborn Sons; "Eldrol" and "Petrosul," obtainable from Pennsylvania Oil Products Refining Co.; Sherwood "Reagent 407," obtainable from Sherwood Refining Co.; "Ultranate No. 2," obtainable from Atlantic Refining Co.; and "SP-1," "SP-302," and "SP-312," obtainable from Stanco Distributors, Inc.

However, the commercially-available, sulfonated petroleum hydrocarbons may be divided on a functional basis into two distinct groups. One of these is the group variously known as "mahogany" acids, "mahogany" soaps, and the like. This group is characterized in that its constituents are generally oil-soluble but water-dispersible. Usually, but not necessarily, these compounds have a deep mahogany color when in solution, which gives rise to the generic designation as "mahogany" compounds.

The other group is generally, but not necessarily, characterized by a green coloration in solution. Hence, compounds of this group are usually referred to as "green sulfonic" acids or "green" soaps. More important than the color distinction, however, is the fact that the so-called "green" compounds are characterized by being water-soluble.

So far as the present invention is concerned, either group, or a mixture thereof, may be used. In using the "green" type of petroleum sulfonates, which are generally, but not necessarily, preferred in the process of the present invention, it will be found that, while they are generally characterized as water-soluble, this is usually of sufficiently high degree that the use of the reagent alone may not always produce the optimum concentration. These green compounds appear to lack certain water-repellent properties which are helpful in making successful concentration. In the process of the present invention, this difficulty is readily overcome by the addition of an amount of a more hydrophobic material. This may be done by adding an oil in suitable quantity or by mixing some of the oil-soluble petroleum sulfonates with the water-soluble type. Any of the commercially-available oils of animal, vegetable, or mineral origin may be used for this purpose. Unsulfonated petroleum derivatives, such as crude oil, kerosene, or fuel oil, are very suitable. Saponifiable oils, such as coconut oil, cotton seed oil, and other glyceride oils may be used. Anionic materials, such as the fatty acids and the like also may be used, provided the gangue constituents are such as not to be floated by these materials. Tall oil, in view of its low cost, is especially useful.

The amounts of reagents used will depend upon the particular group chosen. Whether the oil-soluble type, water-soluble type, or a mixture, is used as the reagent, it will be found that about 0.5-5.0 pounds per ton of ore to be treated will take care of all but the exceptional cases. Ordinarily, however, about 2-4 pounds will be found to constitute a good average practice. In using

the supplemental oiling agent, it will generally be found that from about 0.5-5.0 pounds per ton is also a good operating range. Usually, about 1-2 pounds per ton will constitute a good average practice.

As was pointed out above, one of the principal objects of the present invention is that the process not be unduly sensitive to the presence of slimes. As compared with the use of cationic reagents, in a cationic circuit, this will be found true of the process of the present invention. However, in order to produce a cleaner product and, in many cases, reduce the reagent consumption, a simple desliming is generally found desirable. This may be carried out in any desired manner, in accordance with conventional practice. Usually, this is done by hydraulic classification. With many samples, it will be found that this has also an additional advantage, in that the smaller particle size fractions, i. e., those below about 200 to 150 mesh, frequently contain a higher proportion of the objectionable quartz than do the larger size fractions, i. e., those from the range of about plus 48 to plus 150 mesh. Therefore, a rough desliming may be of assistance in removing some of this fraction.

In general, the process of the invention is relatively simple. The material to be treated is usually reduced to a size suitable for feed to the froth flotation operation, if this is necessary. In general, this will constitute reducing the material to about minus 48 mesh. The resultant particulate material is pulped in water and deslimed, if such an operation is to be used. The use of caustic in the desliming operation is found to be helpful, but not essential. The deslimed sands are then usually conditioned with the flotation reagents. The conditioning is usually, but not necessarily, carried out at approximately pulp flotation density. Generally this constitutes some 18-25% solids. A rougher flotation is then carried out, and this is generally followed by a cleaner float and, generally, a second cleaner float. In the cleaner floatations, it is usually desirable to add a small amount of additional frother, in order to produce the best results. In addition, if, through dilution, there is not sufficient acid to maintain the desired pH, a small amount of make-up acid may be used.

It is believed that the invention will be more readily understood in conjunction with the following examples. These are given as illustrative only, and not by way of limitation. Except as otherwise noted, all parts are considered to be parts by weight. In reporting the following examples, the reagents have been given alphabetical designations, in order to simplify the tables. In the tables, the following reagent designations are used:

- A, sodium hydroxide
- B, sulfuric acid
- C, technical grade alum
- D, commercial alcoholic frother averaging from 7-8 carbon atoms
- E, commercial aliphatic amines mixture averaging 18 carbon atoms
- F, commercial water-soluble "green" petroleum sulfonate
- G, 22° Baumé fuel oil
- H, a commercial diaryl dithiophosphate containing 5-10% thiocarbanilid
- I, commercial steam-distilled pine oil.

It should also be noted, in conjunction with the beneficiation of this material, that the density

improvement is one of the critical factors. Commercially, it is of equal importance with the mica recovery.

#### EXAMPLE 1

A muscovite ore sample, having a density of 58.3 pounds per cubic foot, was subjected to the flotation operation with the reagents outlined in the following Table I. This is a good representation of ordinary, average practice, as conducted in the art, using cationic-type flotation. A clean mica concentrate, amounting to 26.2% by weight of the original sample, and having a density of 40.6 pounds per cubic foot, was obtained. This concentrate contained about 74% mica and 26% quartz. Of the cleaner concentrate, 22.1% of the

mesh, containing 97% mica and 3% quartz; 50.1% by weight was minus 150 mesh and contained 93% mica and 7% quartz. If a greater recovery is required, it can be done by taking advantage of the third cleaner float, which was added in this example. Combining the clean mica concentrate with the third cleaner tail, a concentrate amounting to 30.4% by weight of the feed, assaying about 94% mica and 6% quartz, is obtained, with a satisfactory density.

#### EXAMPLE 3

A sample of lepidolite ore was subjected to flotation, using the conditions and reagents shown in the following Table III.

Table III

| Material                | Time, Min. | Percent Solids | pH    | Reagents |       |       |       |       |
|-------------------------|------------|----------------|-------|----------|-------|-------|-------|-------|
|                         |            |                |       | A        | B     | C     | D     | E     |
| Grind (No Desliming.)   | 2.25       | 54             | ----- | 1.0      | ----- | ----- | ----- | ----- |
| Condition Sand          | 2.0        | 23             | ----- | 2.0      | 1.0   | ----- | ----- | ----- |
| Flotation               | 6.0        | 23             | 5.0   | -----    | 0.132 | 0.125 | ----- | ----- |
| First Cleaner Flotation | 3.0        | -----          | 6.0   | -----    | 0.064 | 0.025 | ----- | ----- |
| Sec. Cleaner Flotation  | 3.0        | -----          | 6.3   | -----    | 0.064 | 0.025 | ----- | ----- |

weight was plus 100 mesh and averaged 99% mica and 1% quartz. About 78% of the concentrate was minus 100 mesh and averaged a mica content of 70% with 30% quartz.

Again, this is a good example of the commercial prior art practice, using an amine in a cationic flotation. A clean mica concentrate is obtained, amounting to 39.5% by weight of the

Table I

| Material                             | Time, Min. | Percent Solids | pH    | Reagents |       |       |       |       |
|--------------------------------------|------------|----------------|-------|----------|-------|-------|-------|-------|
|                                      |            |                |       | A        | B     | C     | D     | E     |
| Grind                                | 2.5        | 54             | ----- | 1.0      | ----- | ----- | ----- | ----- |
| Deslime                              | -----      | -----          | ----- | -----    | ----- | ----- | ----- | ----- |
| Condition Sand                       | 2.0        | 23             | ----- | 1.0      | 1.0   | ----- | ----- | ----- |
| Flotation                            | 6.0        | 23             | 4.3   | -----    | 0.132 | 0.125 | ----- | ----- |
| First Cleaner Flotation <sup>1</sup> | 3.0        | -----          | 5.4   | -----    | 0.064 | 0.025 | ----- | ----- |
| Sec. Cleaner Flotation               | 3.0        | -----          | 6.3   | -----    | 0.064 | 0.025 | ----- | ----- |

<sup>1</sup> Reagents added after 1½.

#### EXAMPLE 2

In order to illustrate the effectiveness of the process of the present invention, another sample of the same ore was subjected to flotation, under the conditions, and using the reagents, shown in the following Table II.

feed, having a density of 38.1 pounds per cubic foot, containing 83% mica and 17% quartz. The ratio of concentration is 2.53:1.0. Of the concentrate, 44.8% was plus 150 mesh, containing 98% mica and 2% quartz; the remainder, 55.2% by weight of minus 150 mesh material, contained 70% mica and 30% quartz.

Table II

| Material                | Time, Min. | Percent Solids | pH    | Reagents |       |       |       |       |
|-------------------------|------------|----------------|-------|----------|-------|-------|-------|-------|
|                         |            |                |       | A        | B     | F     | G     | I     |
| Grind                   | 2.5        | 60             | ----- | 1.0      | ----- | ----- | ----- | ----- |
| Deslime                 | -----      | -----          | ----- | -----    | ----- | ----- | ----- | ----- |
| Condition Sand          | 1.75       | 70             | ----- | 1.6      | 4.0   | 2.1   | ----- | ----- |
| Flotation               | 3.0        | 20             | 3.2   | -----    | ----- | 0.07  | ----- | ----- |
| First Cleaner Flotation | 2.5        | -----          | ----- | -----    | ----- | 0.03  | ----- | ----- |
| Sec. Cleaner Flotation  | 2.5        | -----          | ----- | 0.4      | ----- | ----- | 0.03  | ----- |
| Third Cleaner Flotation | 2.5        | -----          | 3.2   | -----    | ----- | ----- | ----- | ----- |

A cleaned mica concentrate, amounting to 26.9% by weight of the feed, and assaying 95% mica and 5% quartz, was obtained. The ratio of concentration was 3.72:1.0. The concentrate contained 49.9% by weight of material plus 150

75 mesh, containing 97% mica and 3% quartz; 50.1% by weight was minus 150 mesh and contained 93% mica and 7% quartz. If a greater recovery is required, it can be done by taking advantage of the third cleaner float, which was added in this example. Combining the clean mica concentrate with the third cleaner tail, a concentrate amounting to 30.4% by weight of the feed, assaying about 94% mica and 6% quartz, is obtained, with a satisfactory density.

#### EXAMPLE 4

Another sample of the same ore was subjected to flotation, under the conditions and using the reagents shown in the following Table IV.

Table IV

| Material              | Time, Min. | Percent Solids | pH  | Reagents |     |     |      |   |
|-----------------------|------------|----------------|-----|----------|-----|-----|------|---|
|                       |            |                |     | A        | B   | F   | G    | H |
| Grind                 | 2.5        | 54             |     | 1.0      |     |     |      |   |
| Deslime               |            |                |     |          |     |     |      |   |
| Condition             | 4.0        | 65             |     | 1.0      | 3.3 | 0.8 | 0.14 |   |
| Flotation             | 3.0        | 23             | 3.5 |          |     |     |      |   |
| 1st Cleaner Flotation | 2.0        |                | 5.8 |          |     |     |      |   |
| 2nd Cleaner Flotation | 2.0        |                | 6.2 |          |     |     |      |   |
| 3rd Cleaner Flotation | 2.0        |                | 2.6 | 1.0      |     |     |      |   |

In this operation, a concentrate amounting to 28.8% by weight, with a ratio of concentration of 3.47s1.0, was obtained. The density was 37.7 pounds per cubic foot, and it contained 98% mica and 2% quartz. Of the concentrate, 51% by weight was plus 150 mesh and 49% was minus 150 mesh. Both fractions contained 98% mica and 2% quartz. This is a notable change from the result in Example 3, in which substantially the same proportions of plus 150 and minus 150 mesh material was obtained, but the minus 150 mesh fraction was very poor grade and of high density.

All the mica ores of the above examples were substantially free of garnet.

I claim:

1. An improved process of beneficiating mica ore which is substantially free of garnet, which comprises forming an aqueous pulp of the size-reduced ore, conditioning the ore pulp with a reagent combination comprising a strong inorganic mineral acid other than hydrofluoric, an oiling agent, a frother, and an anionic collector selected from the group consisting of water-soluble sulfonated petroleum hydrocarbons of the green acid type, water-insoluble petroleum sulfonates of the mahogany acid type, and mixtures thereof, obtained in the refining of lubricating oil stocks, and the water-soluble salts of such sulfonates; subjecting the conditioned ore to aeration and agitation at a pH of less than 6 and collecting the purified mica as a froth concentrate, substantially free of gangue.

2. An improved process of beneficiating mica ore which is substantially free of garnet, which comprises desliming the size-reduced ore, forming an aqueous pulp of the deslimed ore, conditioning the pulp with a reagent combination comprising a strong inorganic mineral acid other than hydrofluoric, an oiling agent, a frother and an anionic collector selected from the group consisting of water-soluble sulfonated petroleum hydrocarbons of the green acid type, water-insoluble petroleum sulfonates of the mahogany acid type and mixtures thereof obtained in the refining of lubricating oil stocks, and the water-soluble salts of such sulfonates; subjecting the conditioned ore to aeration and agitation at a pH of less than 6 and collecting the purified mica as a froth concentrate, substantially free of gangue.

3. An improved process of beneficiating mica ore which is substantially free of garnet, which comprises forming an aqueous pulp of the size-reduced ore, conditioning the ore pulp with a reagent combination comprising sulfuric acid, an oiling agent, a frother, and an anionic collector selected from the group consisting of water-

soluble sulfonated petroleum hydrocarbons of the green acid type, water-insoluble petroleum sulfonates of the mahogany acid type and mixtures thereof obtained in the refining of lubricating oil stocks, and the water-soluble salts of such sulfonates; subjecting the conditioned ore to aeration and agitation at a pH of less than 6 and collecting the purified mica as a froth concentrate, substantially free of gangue.

4. An improved process of beneficiating mica ore which is substantially free of garnet, which comprises forming an aqueous pulp of the size-reduced ore, conditioning the ore pulp with a reagent combination comprising sulfuric acid, fuel oil, a frother, and an anionic collector selected from the group consisting of water-soluble sulfonated petroleum hydrocarbons of the green acid type, water-insoluble petroleum sulfonates of the mahogany acid type and mixtures thereof obtained in the refining of lubricating oil stocks, and the water-soluble salts of such sulfonates; subjecting the conditioned ore to aeration and agitation at a pH of less than 6 and collecting the purified mica as a froth concentrate substantially free of gangue.

5. An improved process of beneficiating mica ore which is substantially free of garnet, which comprises forming an aqueous pulp of the ore which has been reduced in size sufficiently to pass through a 35-mesh screen, conditioning the ore pulp with a reagent combination comprising sulfuric acid, fuel oil, a frother, and an anionic collector selected from the group consisting of water-soluble sulfonated petroleum hydrocarbons of the green acid type, water-insoluble petroleum sulfonates of the mahogany acid type and mixtures thereof obtained in the refining of lubricating oil stocks, and the water-soluble salts of such sulfonates; subjecting the conditioned ore to aeration and agitation at a pH of less than 6 and collecting the purified mica as a froth concentrate, substantially free of gangue.

ELMER WILLIAM GIESEKE.

#### References Cited in the file of this patent

#### UNITED STATES PATENTS

| Number    | Name            | Date          |
|-----------|-----------------|---------------|
| 2,043,192 | Christmann      | June 2, 1936  |
| 2,257,808 | Phelps          | Oct. 7, 1941  |
| 2,303,962 | Tartaron et al. | Dec. 1, 1942  |
| 2,410,377 | Booth et al.    | Oct. 29, 1946 |
| 2,410,770 | Booth et al.    | Nov. 5, 1946  |
| 2,428,763 | Booth et al.    | Oct. 7, 1947  |
| 2,433,258 | Booth et al.    | Dec. 23, 1947 |

#### OTHER REFERENCES

Mining Technology, November 1944, T. P. 1754, pages 537-538.